

Aug. 23, 1960

B. H. CARROLL ET AL

2,950,196

SUPERSENSITIZATION OF PHOTOGRAPHIC EMULSIONS USING TRIAZINES

Filed Oct. 12, 1955

Fig. 1



Fig. 2



Fig. 3



JOHN SPENCE  
BURT H. CARROLL  
JEAN E. JONES  
INVENTORS

BY *Daniel I. Mayne*

*Lawrence H. Willis*  
ATTORNEYS

# United States Patent Office

2,950,196

Patented Aug. 23, 1960

1

2,950,196

## SUPERSENSITIZATION OF PHOTOGRAPHIC EMULSIONS USING TRIAZINES

Burt H. Carroll, Jean E. Jones, and John Spence, Rochester, N.Y., assignors to Eastman Kodak Company, Rochester, N.Y., a corporation of New Jersey

Filed Oct. 12, 1955, Ser. No. 540,054

20 Claims. (Cl. 96—100)

This invention relates to photographic silver halide emulsions useful in color photography and photographic silver halide emulsions containing dicarbocyanine dyes, and as supersensitizers therefor, triazine compounds.

It is known in the art of making photographic emulsions that certain dyes of the cyanine class alter the sensitivity of photographic emulsions of the gelatinosilver-halide kind, when the dyes are incorporated in the emulsions. It is also known that the sensitization produced by a given dye varies somewhat with the type of emulsion in which the dye is incorporated. Furthermore, the sensitization of a given emulsion by a given dye may be altered by varying the conditions in the emulsion. For example, the sensitization may be increased by increasing the silver ion concentration or decreasing the hydrogen ion concentration (i.e., increasing the alkalinity) or both. Thus, sensitization can be increased by bathing plates, coated with a spectrally sensitized emulsion, in water or in aqueous solutions of ammonia. Such a process of altering the sensitivity of a sensitized emulsion by increasing the silver ion concentration and/or by decreasing the hydrogen ion concentration is commonly called "hypersensitization." Hypersensitized emulsions have generally poor keeping qualities.

We have now found another means of altering the sensitivity in emulsions containing dicarbocyanine dyes. Since the conditions in the emulsion, i.e., the hydrogen ion and/or the silver ion concentration undergo little or no change in our method, we shall designate our method as a kind of supersensitization.

It is, therefore, an object of our invention to provide photographic emulsions containing dicarbocyanine dyes and, as supersensitizers therefor, triazine compounds. Another object is to provide a process for preparing these supersensitized emulsions. Still another object is to provide photographic emulsions containing triazine compounds which are especially useful in color photography. Other objects will become apparent from a consideration of the following description and examples.

The dicarbocyanine dyes which are useful in practicing our invention can advantageously be represented by the following general formula:

I.



wherein R and R<sub>1</sub> each represents an alkyl group (such as methyl, ethyl,  $\beta$ -hydroxyethyl, carboxymethyl,  $\beta$ -carboxyethyl, carbomethoxymethyl, carbethoxymethyl, etc., n represents a positive integer of from 1 to 2, X represents an acid radical, such as chloride, iodide, bromide, perchlorate, p-toluenesulfonate, benzenesulfonate, ethylsulfate, methylsulfate, etc., Z represents the non-metallic atoms necessary to complete a heterocyclic nucleus containing from 5 to 6 atoms in the heterocyclic ring, e.g., a heterocyclic nucleus of the benzothiazole series (e.g., benzothiazole, 4-chlorobenzothiazole, 5-chlorobenzothiazole, 6-chlorobenzothiazole, 7-chlorobenzothiazole, 4-

2

methylbenzothiazole, 5-methylbenzothiazole, 6-methylbenzothiazole, 5-bromobenzothiazole, 6-bromobenzothiazole, 4-phenylbenzothiazole, 5-phenylbenzothiazole, 4-methoxybenzothiazole, 5-methoxybenzothiazole, 6-methoxybenzothiazole, 6-iodobenzothiazole, 5-iodobenzothiazole, 4-ethoxybenzothiazole, 5-ethoxybenzothiazole, 5,6-dimethylbenzothiazole, 5-hydroxybenzothiazole, 6-hydroxybenzothiazole, etc.), a heterocyclic nucleus of the naphthothiazole series (e.g.,  $\alpha$ -naphthothiazole,  $\beta$ -naphthothiazole, 7-methoxy- $\alpha$ -naphthothiazole, 8-methoxy- $\alpha$ -naphthothiazole, 5-methoxy- $\beta$ -naphthothiazole, 5-ethoxy- $\alpha$ -naphthothiazole, etc.), a heterocyclic nucleus of the benzoselenazole series (e.g., benzoselenazole, 5-chlorobenzoselenazole, 6-methoxybenzoselenazole, 5-methoxybenzoselenazole, etc.), a heterocyclic nucleus of the naphthoselenazole series (e.g.,  $\alpha$ -naphthoselenazole,  $\beta$ -naphthoselenazole, etc.), a heterocyclic nucleus of the benzoxazole series (e.g., benzoxazole, 5-hydroxybenzoxazole, 6-hydroxybenzoxazole, 5-chlorobenzoxazole, 5-methoxybenzoxazole, 6-methoxybenzoxazole, 5-phenylbenzoxazole, 5-bromobenzoxazole, etc.), a heterocyclic nucleus of the naphthoxazole series (e.g.,  $\alpha$ -naphthoxazole,  $\beta$ -naphthoxazole, etc.), a heterocyclic nucleus of the 2-quinoline series (e.g., 2-quinoline, 6-methyl-2-quinoline, 7-methyl-2-quinoline, 8-methyl-2-quinoline, 6-chloro-2-quinoline, 8-chloro-2-quinoline, 4-chloro-2-quinoline, 5-ethoxy-2-quinoline, 6-ethoxy-2-quinoline, 7-ethoxy-2-quinoline, 6-hydroxy-2-quinoline, 7-hydroxy-2-quinoline, 6-methoxy-2-quinoline, etc.), a heterocyclic nucleus of the 4-quinoline series (e.g., 4-quinoline, 6-methoxy-4-quinoline, 7-methyl-4-quinoline, 8-methyl-4-quinoline, etc.), a heterocyclic nucleus of the benzimidazole series (e.g., benzimidazole, 5-chlorobenzimidazole, 5,6-dichlorobenzimidazole, 1,7-trimethylenebenzimidazole, etc.), and a heterocyclic nucleus of the 5,6-benzoquinoline series (e.g., 5,6-benzo-2-quinoline, etc.), and Z<sub>1</sub> represents the non-metallic atoms necessary to complete a heterocyclic nucleus selected from the group consisting of those of the benzoxazole series (e.g., such as those defined by Z above), those of the naphthoxazole series (e.g., such as those defined by Z above), those of the benzoselenazole series (e.g., such as those defined by Z above), those of the naphthoselenazole series (e.g., such as those defined by Z above), those of the benzothiazole series (e.g., such as those defined by Z above), and those of the naphthothiazole series (e.g., such as those defined by Z above).

The triazine compounds useful in practicing our invention comprise symmetrical triazine (i.e., 1,3,5-triazine) compounds, which can be simple triazine compounds or more complex polynuclear compounds. Such compounds comprise simple s-triazine compounds, such as those having an arylamino or substituted arylamino substituent, an alkylamino substituent (particularly those substituents having seven or more carbon atoms), a heterocyclyl substituent, etc., or more complex structures, such as the bis-triazinylaminobenzyl compounds, bis-triazinylaminocarbazole compounds, etc. The supersensitizing effect of these compounds appears to be a function of the s-triazine ring, as evidenced by the variety of compounds having this structure which have been found useful in our invention.

The bis-triazinylaminobenzyl compounds useful in practicing our invention comprise those compounds represented by the following general formula:

II.



wherein R<sub>6</sub>, R<sub>7</sub>, R<sub>2</sub>, and R<sub>3</sub> each represents a hydrogen atom, or a substituent group, such as hydroxyl, aryloxy (e.g., phenoxy, o-toloxyl, p-sulfophenoxyl, etc.), alkoxy (e.g., methoxyl, ethoxyl, etc.), a halogen atom (e.g., chlorine, bromine, etc.), a heterocyclic radical (e.g., morpholinyl, piperidyl, etc.), an alkylthio group (e.g., methylthio, ethylthio, etc.), an arylthio group (e.g., phenylthio, tolylthio, etc.), a heterocyclthio group (e.g., benzothiazylthio, etc.), an amino group, an alkylamino group (e.g., methylamino, ethylamino, propylamino, dimethylamino, diethylamino, dodecylamino, cyclohexylamino,  $\beta$ -hydroxyethylamino, di- $\beta$ -hydroxyethylamino,  $\beta$ -sulfoethylamino, etc.), an arylamino group (e.g., anilino, o-, m-, and p-sulfoanilino, o-, m-, and p-chloroanilino, o-, m-, and p-anisylamino, o-, m-, and p-toluidino, o-, m-, and p-carboxyanilino, hydroxyanilino, sulfonaphthylamino, o-, m-, and p-aminoanilino, p-acetamidoanilino, etc.), a heterocyclamino group (e.g., 2-benzothiazylamino, 2-pyridylamino, etc.), etc., and R<sub>4</sub> and R<sub>5</sub> each represents a hydrogen atom or a water-solubilizing group, such as sulfo, carboxyl, etc. (as well as alkali metal or amine salts of such groups). Listed below are representative compounds selected from those represented by Formula II, although our invention is not limited in any sense to these particular compounds. While the structural formulas are included for only the first three compounds, it is to be understood that the same numbering system is employed throughout the specification.



- (3a) 4,4'-bis(4-chloro-6-trimethylolmethylamino-s-triazin-2-ylamino)biphenyl-2,2'-disulfonic acid  
 (4) 4,4'-bis[4-(4'-sulfoanilino)-6-( $\beta$ -hydroxyethyl)amino-s-triazin-2-ylamino]biphenyl-2,2'-disulfonic acid  
 (5) 4,4'-bis(4,6-dianilino-s-triazin-2-ylamino)biphenyl-2,2'-disulfonic acid  
 (6) 4,4'-bis[4-phenoxo-6-( $\beta$ -hydroxyethyl)amino-s-triazin-2-ylamino]biphenyl-2,2'-disulfonic acid  
 (7) 4,4'-bis[4-anilino-6-hydroxy-s-triazin-2-ylamino]biphenyl-2,2'-disulfonic acid  
 (8) 4,4'-bis[4-N-morpholinyl-6-(4'-sulfoanilino)s-triazin-2-ylamino]biphenyl-2,2'-disulfonic acid  
 (9) 4,4'-bis[4-chloro-6-di( $\beta$ -hydroxyethyl)amino-s-triazin-2-ylamino]biphenyl-2,2'-disulfonic acid  
 (10) 4,4'-bis[4-anilino-6-( $\beta$ -hydroxyethyl)amino-s-triazin-2-ylamino]biphenyl-2,2'-disulfonic acid

The bis-triazinylaminocarbazole compounds useful in practicing our invention comprise those represented by the following general formula, although related compounds having a substituent on the nitrogen atom of the carbazole nucleus can also be employed to advantage.



wherein R<sub>2</sub>, R<sub>3</sub>, R<sub>4</sub>, R<sub>5</sub>, R<sub>6</sub>, and R<sub>7</sub> each have the values given above. Representative of the compounds represented by Formula III above are those listed below. Although the structural formulas are given for the first two compounds, the same numbering system was employed throughout.



30

35

30

35



60

65

- (13) 2,8-bis[4-(4-sulfoanilino)-6-piperidino-s-triazin-2-ylamino]carbazole  
 (14) 2,8-bis[4-anilino-6-( $\beta$ -hydroxyethyl)amino-s-triazin-2-ylamino]carbazole  
 (15) 2,8-bis[4-chloro-6-di( $\beta$ -hydroxyethyl)amino-s-triazin-2-ylamino]carbazole

More simple triazine compounds which can be em-

ployed in practicing our invention comprise those represented by the following general formula:

IV.



wherein R<sub>2</sub>, R<sub>3</sub> and R<sub>6</sub> each have the values given above. Representative compounds selected from those of Formula IV comprise the following. While only the first four compounds are identified by structural formulas, the same numbering system is employed throughout.

(16)



2-(3-sulfoanilino)-6-hydroxy-4-(β-hydroxyethyl)amino-s-triazine

(17)



2,4-diamino-6-(2-furyl)-s-triazine

(18)



1,4-bis[4-(4-anilino-6-β-hydroxyethylamino-s-triazin-2-ylamino)-2-sulfostyryl]benzene

(19)



4,4'-bis(4,6-di(β-hydroxyethylamino)-s-triazin-2-yl)benzidine-2,2'-disulfonic acid

(20) 4,4'-bis[4,6-di(β-hydroxyethylamino)-s-triazin-2-ylamino]diphenylamine

(21) 2-chloro-4,6-di(β-hydroxyethylamino)-s-triazine

(22) 2-laurylamino-4,6-di(4-sulfoanilino)-s-triazine

(23) 2,4-diamino-6-(2-hydroxyphenyl)-s-triazine

(24) 2,4-diamino-6-methyl-s-triazine

(25) 2,4-diamino-6-(3-hydroxy-2-naphthyl)-s-triazine

(26) 2,4-diamino-6-(2-hydroxystyryl)-s-triazine

(27) 2,4-diamino-6-(2-hydroxy-3-nitrophenyl)-s-triazine

(28) 2-amino-4-n-aminyl-6-N-morpholinyl-s-triazine

(29) 2-amino-4-(4-chloroanilino)-6-methyl-s-triazine

(30) 2-amino-4-N-morpholinyl-6-phenyl-s-triazine

(31) 2-(4-anisyl)-4,6-di(ethylamino)-s-triazine

(32) 2,4-diamino-6-decyloxy-s-triazine

(33) 2,4-diamino-6-hendecyl-s-triazine

(33a) 2,4-dichloro-6-(2-pyridylamino)-s-triazine

(34) 2-(4-chloroanilino)-4-diethylaminoethylamino-6-methyl-s-triazine

(35) 2-amino-4-chloro-6-(1-piperidyl)-s-triazine

(36) 2-amino-4-(2-pyridylamino)-s-triazine

(37) 2,4-diamino-6-(5-pyrimidyl)-s-triazine

(38) 2,4-diamino-6-(4-quinolyl)-s-triazine

(39) 2,4-diamino-6-(2-thienyl)-s-triazine

(40) 2-amino-4-n-butylamino-6-(1-ethyl)amyl-s-triazine

(41) 2-(2-benzothiazylamino)-4,6-dichloro-s-triazine

(42) 2-(2-benzothiazylamino)-4,6-dihydroxy-s-triazine

According to our invention, we incorporate one or more of the dicarbocyanine dyes represented by Formula I above with one or more triazine compounds, such as those represented by Formulas II, III or IV above. Our invention is particularly directed to the ordinarily employed gelatino-silver-halide emulsions. However, our supersensitizing combinations can be employed in silver halide emulsions in which the carrier is other than gelatin, e.g., a resinous substance or cellulosic material which has no deteriorating effect on the light-sensitive materials. The dicarbocyanine dyes and triazine compounds can be employed in various concentrations depending upon the effects desired.

Ordinarily, the optimum or near optimum concentration of the dicarbocyanine dyes which we employ in practicing our invention is of the order of from 0.010 to 0.30 g. per mol. of silver halide in the emulsion.

The triazine compounds which we employ in our invention can advantageously be employed at a concentration of from about 0.03 to 10.0 g. per mol. of silver halide in the emulsion.

In general, the ratio of concentration of dicarbocyanine dye to triazine compound can vary rather widely in our combinations, e.g., from 1:1 to 1:300 (by weight) in many cases.

The methods of incorporating sensitizing dyes in silver halide emulsions are well known to those skilled in the art. The triazine compounds can be directly dispersed in the emulsions, or they can be dissolved in water (or

an organic solvent, such as methanol, ethanol, etc., where the water-solubility is not sufficiently great) and added in the form of their solutions. While the dicarbocyanine dyes can be directly dispersed in the emulsions, it is convenient to add the same in the form of solutions in appropriate solvents. Methanol, ethanol, pyridine, and the like have proven satisfactory for many of the dyes of Formula I. Mixtures of solvents, e.g., pyridine diluted with methanol or acetone, can also be used. The dicarbocyanine dyes and triazine compounds are dispersed in the finished emulsions and should be uniformly distributed throughout the emulsions. The following procedure is satisfactory: Stock solutions of the dicarbocyanine dyes and triazine compounds are prepared by dissolving the same in appropriate solvents as described above. Then, to the flowable gelatino-silver-halide emulsion, the desired amounts of the stock solution of one of the dyes (or triazine compounds) are slowly added, while stirring the emulsion. Stirring is continued until the dye is thoroughly incorporated in the emulsion. Then the desired amount of the stock solution of the triazine compound (or dye, if triazine compound has been added first) is slowly added to the emulsion, while stirring. Stirring is continued until the second solution is thoroughly incorporated. The supersensitized emulsion can then be coated out on a suitable support, such as glass, cellulose derivative film, resin film, or paper, to a suitable thickness and allowed to dry. The details of

such coating methods are well known to those skilled in the art. The foregoing procedures and proportions are to be regarded only as illustrative. Clearly, our invention is directed to any silver halide emulsion containing a combination of the aforesaid dicarbocyanine dyes and triazine compounds whereby a supersensitizing effect is obtained.

The following examples will serve to illustrate further the manner of practicing our invention.

In Table I below, to different portions of the same batch of photographic gelatino-silver-bromide emulsion were added (1) a dicarbocyanine dye, such as those represented by Formula I above, and (2) a combination of the dicarbocyanine dye and a triazine compound (in neutral aqueous solution). Then the emulsions were held at about 50-52° C. for a short time and coated on a support, chill set, and dried. After exposure through a Wratten No. 25 filter, i.e., a filter which transmits substantially no light of wavelength shorter than about 580 m $\mu$ , in an Eastman Type IB sensitometer, the film strips were processed for 4 minutes in a developer having the following composition:

|                                | G.   |
|--------------------------------|------|
| N-methyl-p-aminophenol sulfate | 2.0  |
| Hydroquinone                   | 8.0  |
| Sodium sulfite (desiccated)    | 90.0 |
| Sodium carbonate (monohydrate) | 52.5 |
| Potassium bromide              | 5.0  |
| Water to make 1 liter.         |      |

The speed (red), gamma and fog for each of the coatings was then measured. The results are recorded in Table I.

TABLE I

| Example | Sensitizing Dye and Addenda (g./mol. AgX)                                          | Red Light Exposure |       |     |
|---------|------------------------------------------------------------------------------------|--------------------|-------|-----|
|         |                                                                                    | Relative Speed     | Gamma | Fog |
| 1       | (a) 3,3'-diethyloxathiadicarbocyanine iodide (.05)                                 | 100                | 4.7   | .06 |
|         | (b) dye (a) (.050) plus compound 1 (4.0)                                           | 465                | 5.6   | .09 |
| 2       | (c) dye (a) (.050) plus compound 2 (4.0)                                           | 485                | 5.1   | .09 |
|         | (d) dye (a) (.050)                                                                 | 100                | 4.5   | .05 |
| 3       | (e) dye (a) (.050) plus compound 2 (4.0)                                           | 535                | 4.5   | .05 |
|         | (f) 3-ethyl-3'- $\beta$ -hydroxyethylxathiadicarbocyanine iodide (.050)            | 240                | 4.9   | .07 |
| 4       | (g) dye (f) (.050) plus compound 2 (4.0)                                           | 735                | 4.8   | .05 |
|         | (h) 3,3'-diethyl-5-phenyloxathiadicarbocyanine-p-toluenesulfonate (.050)           | 37                 | 3.0   | .08 |
| 5       | (i) dye (h) (.050) plus compound 2 (4.0)                                           | 370                | 4.7   | .06 |
|         | (j) 3-ethyl-3'- $\beta$ -hydroxyethyl-5-phenyloxathiadicarbocyanine bromide (.050) | 137                | 5.3   | .07 |
| 6       | (k) dye (j) (.050) plus compound 2 (4.0)                                           | 640                | 4.5   | .06 |

In the above table, the coatings of Examples 1 and 2 were made from the same batch of emulsion and the coatings of Examples 3, 4, 5 and 6 were made from the same batch of emulsion. No measurements of coatings containing only the triazine compound alone are given, since numerous coatings at the concentrations used in the table have shown that these triazine compounds alone have little or no measureable sensitizing effect on the emulsions.

Our invention is primarily directed to the ordinarily employed gelatino-silver-halide developing-out emulsions, e.g., gelatino-silver-chloride, -chlorobromide, -chloroiodide, -chlorobromiodide, -bromide and -bromiodide developing-out emulsions. Emulsions which form the latent image mostly inside the silver halide grains, such as the emulsions set forth in U.S. Patent 2,456,956, dated December 21, 1948, can also be employed in practicing our invention.

The emulsions prepared in accordance with our invention can be coated in the usual manner on any suitable support, e.g., glass, cellulose nitrate film, cellulose acetate film, polyvinyl-acetal resin film, paper or metal.

Photographic silver halide emulsions, such as those listed above, containing the supersensitizing combinations of our invention can also contain such addenda as chemi-

cal sensitizers, e.g., sulfur sensitizers (e.g., allyl thiocarbamide, thiourea, allylisothiocyanate, cystine, etc.), various gold compounds (e.g., potassium chloroaurate, auric trichloride, etc.) (see U.S. Patents 2,540,085; 2,597,856 and 2,597,915), various palladium compounds, such as palladium chloride (U.S. 2,540,086), potassium chloropalladate (U.S. 2,598,079), etc., or mixtures of such sensitizers; antifoggants, such as ammonium chloroplatinate (U.S. 2,566,245), ammonium chloroplatinite (U.S. 2,566,263), benzotriazole, nitrobenzimidazole, 5-nitroindazole, benzidine, mercaptans, etc. (see Mees—“The Theory of the Photographic Process,” Macmillan Pub., page 460), or mixtures thereof; hardeners, such as formaldehyde (U.S. 1,763,533), chrome alum (U.S. 1,763,533), glyoxal (U.S. 1,870,354), dibromacrolein (Br. 406,750), etc; color couplers, such as those described in U.S. Patent 2,423,730, Spence and Carroll U.S. Patent 2,640,776, etc.; or mixtures of such addenda. Dispersing agents for color couplers, such as those set forth in U.S. Patents 2,322,027 and 2,304,940, can also be employed in the above-described emulsions.

Such silver halide emulsions can also contain thiazolines or other ultraviolet absorbing compounds, such as those described in the copending application Serial No. 419,239, filed March 29, 1954 in the name of G. W. Sawdey (now U.S. Patent 2,739,888, issued March 27, 1956). While certain emulsion addenda, such as certain ultraviolet compounds, and certain color-forming compounds cause de-sensitization or un-sensitizing effects, it has been found that the new combinations of our invention largely overcome such effects. Typical color-forming compounds which can be so employed include those in U.S. Patent 2,322,027 and the following:

## COUPLER

- (1) 1 - hydroxy - 2-[ $\delta$ -(2',4'-di-tert.amylphenoxy - n - butyl)-naphthamide (U.S. Patent 2,474,293)
- (2) 1 - hydroxy - 4 - phenylazo - 4' - (p - tert.-butylphenoxy)-2-naphthaniide (U.S. Patent 2,521,908)
- (3) 2 - (2,4 - di - tert.amylphenoxyacetamino) - 4,6-dichloro-5-methyl phenol (Graham U.S. application Serial No. 285,544, now U.S. Patent 2,725,291)
- (4) 2 - ( $\alpha$ -2,4-di-tert.amylphenoxy - n - butyrylarnino) - 4,6-dichloro-5-methyl phenol
- (5) 6 - { $\alpha$  - {4 - [ $\alpha$  - (2,4-di-tert.amylphenoxy)butyramido] - phenoxy}acetamido} - 2,4 - dichloro - 3 - methyl phenol
- (6) 2 - [3' - (2',4'' - diamylphenoxy) - acetamido]-benzamido - 4 - chloro - 5 - methyl phenol
- (7) 1 - (2',4',6' - trichlorophenyl) - 3 - [3''-(2'',4''' - di-tert.-amylphenoxyacetamido) - benzamido] - 5 - pyrazolone (U.S. Patent 2,600,788)
- (8) 1 - (2',4',6 - trichlorophenyl) - 3 - [3''-(2'',4''' - di-tert. - amylphenoxyacetamido) - benzamido] - 4 - (p-methoxyphenylazo)-5-pyrazolone
- (9) N - (4 - benzoylacetaminobenzenesulfonyl) - N - ( $\gamma$ -phenylpropyl)-p-toluidine (U.S. Patent 2,298,443)
- (10)  $\alpha$  - o - methoxybenzoyl -  $\alpha$  - chloro - 4 - [ $\alpha$  - (2,4-di-tert. - amylphenoxy) - n - butyramido] - acetanilide

- (McCrossen U.S. application Serial No. 295,806, now U.S. Patent 2,728,658, issued December 27, 1955)
- (11)  $\alpha$  - {3 - [ $\alpha$  - (2,4-di-tert.amylphenoxy)acetamido] - benzoyl}-2-methoxyacetanilide
- (12) 3-benzoylacetamido - 4 - methoxy - 2',4'-di-tert.-amylphenoxy acetanilide
- (13) 4-benzoylacetamido - 3 - methoxy - 2',4' - di-tert.-amylphenoxy acetanilide

The following table and examples will serve to illustrate the beneficial effects of our new supersensitizing combinations when employed in a photographic emulsion containing a dispersion of a coupler or color-forming compound. In Table II these effects are illustrated for the same batches of emulsions employed in arriving at the data in Table I. To a separate portion of each of the emulsions set forth under Table I above was added

The coatings in the following examples were prepared and processed exactly as described for the coatings of Table I, except that exposure was made in an intensity scale sensitometer (using Wratten No. 25 filter). The emulsions were coated on a glass plate and chill set before exposure. The coatings of Examples 13, 14 and 15 were made from the same batch of gelatino-silver-bromide emulsion, the coatings of Examples 16, 17, 18, 19, 20, 21 and 22 were made from the same batch of gelatino-silver-bromide emulsion, the coatings of Example 23 were made from the same batch of gelatino-silver-bromide emulsion, the coatings of Examples 24 and 25 were made from the same batch of gelatino-silver-bromide emulsion, and the coatings of Examples 26 and 27 were made from the same batch of gelatino-silver-bromide emulsion.

TABLE III

| Example | Sensitizing Dye and Addenda (g./mol. AgX)   | Red Light Exposure |       |     |
|---------|---------------------------------------------|--------------------|-------|-----|
|         |                                             | Relative Speed     | Gamma | Fog |
| 13      | {(l) dye (a) (.050)                         | 100                | 4.2   | .06 |
|         | {(m) dye (a) (.050) plus compound 18 (4.0)  | 380                | 5.3   | .07 |
| 14      | {(n) dye (a) (.050) plus compound 19 (4.0)  | 270                | 5.3   | .08 |
| 15      | {(o) dye (a) (.050) plus compound 20 (4.0)  | 280                | 4.6   | .07 |
| 16      | {(p) dye (a) (.050)                         | 100                | 4.8   | .06 |
|         | {(q) dye (a) (.050) plus compound 21 (4.0)  | 230                | 4.4   | .10 |
| 17      | {(r) dye (a) (.050) plus compound 22 (4.0)  | 370                | 4.6   | .06 |
| 18      | {(s) dye (a) (.050) plus compound 23 (4.0)  | 245                | 4.4   | .07 |
| 19      | {(t) dye (a) (.050) plus compound 24 (4.0)  | 169                | 4.6   | .10 |
| 20      | {(u) dye (a) (.050) plus compound 25 (4.0)  | 185                | 4.1   | .10 |
| 21      | {(v) dye (a) (.050) plus compound 26 (4.0)  | 670                | 4.1   | .43 |
| 22      | {(w) dye (a) (.050) plus compound 27 (4.0)  | 161                | 4.5   | .12 |
| 23      | {(x) dye (a) (.050)                         | 100                | 4.8   | .06 |
|         | {(y) dye (a) (.050) plus compound 11 (4.0)  | 465                | 4.7   | .06 |
| 24      | {(z) dye (a) (.050)                         | 100                | 4.5   | .06 |
|         | {(a') dye (a) (.050) plus compound 12 (4.0) | 210                | 4.1   | .06 |
| 25      | {(b') dye (a) (.050) plus compound 13 (4.0) | 445                | 5.2   | .07 |
| 26      | {(c') dye (a) (.050)                        | 100                | 3.9   | .04 |
|         | {(d') dye (a) (.050) plus compound 41 (4.0) | 885                | 1.8   | .06 |
| 27      | {(e') dye (a) (.050) plus compound 42 (4.0) | 285                | 4.5   | .06 |
| 27(a)   | {(e') dye (a) (.050) plus compound 3a (4.0) | 205                | 5.2   | .06 |

a coupler dispersion containing coupler No. 5 of the above list. The emulsions were then held for the times indicated in the table below. After exposure and development of the coatings (exactly as in Table I), the relative red speed, gamma and fog for the coatings was measured. The results are given in Table II below. (The example numbers referred to in the table are those of Table I.)

TABLE II

| Example | Dispersion Plus Emulsion of- | Holding Time (Minutes) | Red Light Exposure |       |     |
|---------|------------------------------|------------------------|--------------------|-------|-----|
|         |                              |                        | Relative Speed     | Gamma | Fog |
| 7       | {Example 1 (a)               | 30                     | 7.9                | .39   | .20 |
|         | {Example 1 (b)               | 30                     | 260                | 3.9   | .24 |
| 8       | Example 2 (c)                | 30                     | 640                | 3.5   | .09 |
| 9       | {Example 3 (d)               | 60                     | 40                 | 1.8   | .09 |
|         | {Example 3 (e)               | 60                     | 485                | 3.6   | .13 |
| 10      | {Example 4 (f)               | 60                     | 14                 | .60   | .16 |
|         | {Example 4 (g)               | 60                     | 500                | 2.9   | .07 |
| 11      | {Example 5 (h)               | 60                     | 38                 | 2.5   | .13 |
|         | {Example 5 (i)               | 60                     | 295                | 3.1   | .15 |
| 12      | {Example 6 (j)               | 60                     | 24                 | 1.6   | .19 |
|         | {Example 6 (k)               | 60                     | 535                | 3.2   | .13 |

In the example below, the emulsion coatings were prepared in exactly the manner as those of Table I, except that the digestion temperature was about 40° C. Each coating contained .05 g./mol. of AgX of dye (a) of Table I. The control contained no triazine compound while the second coating contained 4.0 g./mol. AgX of compound 16. The results follow:

| Example                        | Red Light Exposure | Example 28 |       |     |
|--------------------------------|--------------------|------------|-------|-----|
|                                |                    | Speed      | Gamma | Fog |
| control                        |                    | 100        | 4.1   | .05 |
| control plus triazine (No. 16) |                    | 535        | 5.3   | .07 |

The data in the following table were obtained from coatings of an ordinary gelatino-silver-bromide emulsion in precisely the manner described for the coatings of Table I. These coatings were also processed in the same manner as those of Table I. The speed (red), gamma and fog for the exposed coatings are given in Table IV below. All coatings were made from the same batch of emulsion.

TABLE IV

| Example | Sensitizing Dye and Addenda (g./mol. AgX)             | Red Light Exposure |       |     |
|---------|-------------------------------------------------------|--------------------|-------|-----|
|         |                                                       | Speed              | Gamma | Fog |
| 29      | {(f') 3,3'-diethylthiadicyanine iodide (.050)         | 5.4                | .76   | .06 |
|         | {(g') dye (f') (.050) plus compound 1 (1.0)           | 24.0               | 2.1   | .06 |
| 30      | {(h') dye (f') (.050) plus compound 18 (1.0)          | 26.0               | 2.4   | .06 |
| 31      | {(i') 3,3'-diethylselenadicarbocyanine bromide (.050) | 5.7                | .96   | .06 |
|         | {(j') dye (i') (.050) plus compound 1 (1.0)           | 18.0               | 2.0   | .06 |
| 32      | {(k') dye (i') (.050) plus compound 18 (1.0)          | 18.5               | 2.5   | .06 |

The dyes represented by Formula I above comprise a well known class of optical sensitizing dyes. While these dyes have been described in the prior art, methods for making them are also described in Carroll, Jones and Spence U.S. application Serial No. 540,052 filed on even date herewith.

The triazine compounds employed in our invention, e.g., those of Formulas II, III and IV above, have, in general, been described in the prior art. The bibenzyl compounds of Formula II and the carbazole compounds of Formula III, for example, can be prepared in exactly the same manner as the stilbene compounds of Serial No. 540,052 by employing the corresponding diamino-bibenzyl and diaminocarbazole compounds. Thus these corresponding diamino compounds can be condensed with cyanuric chloride (step 1 of Serial No. 540,052), followed by condensation with ammonia or an amine (step 2), and/or hydrolysis (step 3) or condensation with further ammonia or amine. See also British Patent 616,523, accepted January 24, 1949 for this method. The preparation of a number of the compounds of Formulas II and III can be summarized as follows:

| Compound | Used in Step 1                     | Used in Step 2                              | Step 3                          |
|----------|------------------------------------|---------------------------------------------|---------------------------------|
| 3a       | 4,4'-bibenzyl-2,2'-disulfonic acid | (trishydroxymethyl)-amino-methane (2 mols.) | omitted.                        |
| 2        | do                                 | $\beta$ -aminoethanol (2 mols.)             | $\beta$ -aminoethanol (2 mols.) |
| 1        | do                                 | hydrolysis                                  | hydrolysis                      |
| 19       | benzidine-2,2'-disulfonic acid     | $\beta$ -aminoethanol (2 mols.)             | $\beta$ -aminoethanol (2 mols.) |
| 11       | 2,8-diaminocarbazole               | sodium sulfonate (2 mols.)                  | sodium sulfonate (2 mols.)      |
| 12       | do                                 | do                                          | morpholine (2 mols.)            |
| 13       | do                                 | do                                          | piperidine (2 mols.)            |
| 20       | 4,4'-diaminodiphenylamine          | $\beta$ -aminoethanol (2 mols.)             | $\beta$ -aminoethanol (2 mols.) |

The diamine compound required to prepare compound 18 was prepared as follows:

p-Nitrotoluene was treated with chlorosulphonic acid to form p-nitrotoluene-2-sulphonylchloride. This compound was converted into its phenylester with sodium phenoxide. This product was condensed with terephthalaldehyde to yield 4':4"-dinitro-1:4-distyrylbenzene-2':2"-disulfonic acid phenylester. The terephthalaldehyde was prepared by the tetrabromination of p-xylol and subsequent hydrolysis of the bromination compound with sulphuric acid.

The 4':4"-dinitro-1:4-distyrylbenzene-2':2"-disulfonic acid phenyl ester was then reduced to the corresponding 4':4"-diamino compound with Raney nickel and the ester hydrolyzed to the free sulfonic acid with aqueous alkali. (British 668,200.)

The triazine compounds represented by Formula IV above comprise many known compounds. While methods for making these compounds are also well known, the following example will serve to illustrate the preparation of one of these compounds.

*Example 33.—2-lauryl amino-4,6-di(4-sulfoanilino)-s-triazine*

One hundred and twenty-four parts of 6-chloro-2,4-di(sodium-p-sulfophenylamino)-3-triazine (prepared as in step 2, using sulfanilic acid and cyanuric chloride) and 92 parts of laurylamine were stirred in dimethylformamide at 145-150° C. for 5-6 hours. The white solid which was collected from the cooled reaction mixture was suspended in water containing 10 parts of sodium hydroxide and extracted with ethyl ether. The water layer was concentrated to dryness, and the remaining solid treated with ethyl ether several times. Eighty-eight parts of a white solid was obtained. The free acid was obtained upon acidification.

Other triazine compounds of Formula IV can be similarly prepared. For example, compound 41 was obtained simply by condensing cyanuric chloride with 2-aminobenzothiazole. Hydrolysis of compound 41 (step 3) gave compound 42.

We have also found that the compounds of the type represented by Formulas II, III and IV above can advantageously be employed in photographic silver halide emulsions, and particularly photographic silver bromide emulsions (negative speed), containing color-forming or coupling compounds of the type described above to prevent or diminish the formation of spontaneous fog which develops upon exposure of the emulsions to high temperatures and humidity. Also, we have found that the s-triazine compounds of our invention have the valuable property of inhibiting the formation of stain which frequently remains after processing of photographic emulsions containing color-forming compounds. The anti-foggant and/or anti-stain action of these compounds appears to be unrelated to the supersensitizing effect shown in the above examples. That is, this anti-foggant or anti-stain action appears to take place regardless of the presence of sensitizing dyes in the emulsions containing the color-forming compounds of the type mentioned above.

The anti-foggant and/or anti-stain action of the s-triazine compounds of our invention appears to be particu-

larly outstanding in the presence of color-forming compounds for the magenta or cyan images, i.e. in the presence of magenta or cyan couplers (e.g. such as the magenta and cyan couplers described in U.S. Patent 2,640,776 mentioned above). The anti-foggant and anti-stain action of the s-triazine compounds of our invention is particularly apparent at concentrations of 1 gram of compound per mole of silver halide, or amounts in excess of 1 gram (e.g., from about 1 to 10 grams per mole of silver halide). It has also been found that the s-triazine compounds of our invention are particularly useful in combination with color couplers of the water-soluble type (such as the couplers described in U.S. application Ser. No. 470,499, filed November 22, 1954) now U.S. Patent 2,808,329, issued October 1, 1957. Such couplers when used in the absence of the s-triazine compounds cause sufficiently high fog to make their use difficult in photographic emulsions. However, when using such couplers in the presence of our s-triazine compounds, the fog is reduced to a considerable degree so that such couplers can be employed from a practical standpoint.

The following example will serve to illustrate the anti-foggant action of our s-triazine compounds when employed in a photographic silver halide emulsion containing a color-forming compound.

*Example 34*

A red sensitive chloro bromide emulsion containing a color coupler, such as coupler No. 5 above, was divided into two batches and these batches coated on cellulose acetate supports and dried. One coating was exposed in an intensity scale sensitometer through a Wratten No. 25 filter, while the second coating was incubated at 120° F. (50% relative humidity) for seven days before exposure. The exposed coatings were then processed as described in Example 46 of our copending application Ser. No. 540,052, filed on even date herewith. The fog measurements for the coating which contained no anti-foggant is compared in the following table with an exact coating which contained 2,4-diamino-6-n-heptadecyl-s-tri-

azine (in the amount shown in the table). The results follow.

| Coating  | Antifoggant<br>(g./mol.<br>AgX) | Original<br>Fog | Incubation<br>Fog (7<br>days/120° F.,<br>50% R.H.) |
|----------|---------------------------------|-----------------|----------------------------------------------------|
| (a)----- | none-----                       | .09             | .23                                                |
| (b)----- | A-----                          | .07             | .10                                                |

A = 2,4-diamino-6-n-heptadecyl-s-triazine.

As shown in the above examples, the compounds of Formulas II, III and IV above are generally employed in neutral aqueous solution, when such compounds contain a free sulfonic acid group. That is, the free acids are at least partially neutralized with sodium hydroxide, potassium hydroxide, sodium carbonate, ammonia, triethylamine, etc. before use in the emulsions. The corresponding sulfonic acid salts result. It is thus possible to adjust the pH of these aqueous solutions so that they are about the same as the pH of the emulsions.

The accompanying drawing illustrates the supersensitizing effect obtained with three of our new combinations in gelatino-silver-bromide emulsions. Each figure of the drawing is a diagrammatic reproduction of one or two (Fig. 1) spectrograms. The sensitivity of the emulsion containing only the dicarbocyanine dye represented by Formula I is represented by the broken line in Fig. 1, while the sensitivity of the same emulsion containing both a dicarbocyanine dye of Formula I and a triazine compound of Formulas III or IV is represented by the solid curve. The sensitizing dye used in Fig. 1 was also employed in the coatings of Figs. 2 and 3, hence curve A of Fig. 1 is not reproduced in Figs. 2 and 3 since it would merely be identical thereto.

In Fig. 1, curve A represents the sensitivity of an ordinary gelatino-silver-bromide emulsion containing 3,3'-diethyloxathiadicarbocyanine iodide, while curve B represents the sensitivity of the same emulsion sensitized with 3,3'-diethyloxathiadicarbocyanine iodide and 2,8-bis[4-(4-sulfoanilino)-6-hydroxy-s-triazine-2-ylamino] carbazole. Sensitometric measurements for coatings prepared in substantially the same manner are given in Example 23 above.

In Fig. 2, curve C represents the sensitivity of an ordinary gelatino-silver-bromide emulsion sensitized with 3,3'-diethyloxathiadicarbocyanine iodide and 2,4-diamino-6-(2-hydroxystyryl)-s-triazine. Sensitometric measurements for coatings prepared in substantially the same manner are given in Example 21 above.

In Fig. 3, curve D represents the sensitivity of an ordinary gelatino-silver-bromide emulsion sensitized with 3,3'-diethyloxathiadicarbocyanine iodide and 6-hydroxy-4-β-hydroxyethylamino-2-(3-sulfoanilino)-s-triazine. Sensitometric measurements for coatings prepared in substantially the same manner are given in Example 28 above.

What we claim as our invention and desire secured by Letters Patent of the United States is:

1. A photographic silver halide emulsion sensitized with a supersensitizing combination of at least one dicarbocyanine dye selected from the class represented by the following general formula:



wherein R and R<sub>1</sub> each represents an alkyl group containing from 1 to 4 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series,

those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, those of the naphthoselenazole series, those of the 2-quinoline series, those of the 4-quinoline series, those of the benzimidazole series, and those of the 5,6-benzoquinoline series, and at least one compound containing at least one s-triazine ring.

2. A photographic silver halide emulsion sensitized with a supersensitizing combination of at least one dicarbocyanine dye selected from the class represented by the following general formula:



wherein R and R<sub>1</sub> each represents an alkyl group containing from 1 to 4 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, those of the naphthoselenazole series, those of the 2-quinoline series, those of the benzimidazole series, and those of the 5,6-benzoquinoline series, and at least one triazine compound selected from the class represented by the following general formula:



wherein R<sub>2</sub>, R<sub>3</sub>, R<sub>6</sub> and R<sub>7</sub> each represents a member selected from the group consisting of a hydrogen atom, a hydroxyl group, an aryloxyl group, an alkoxy group, a halogen atom, a heterocyclic radical, an alkylthio group, an arylthio group, and an amino group, and R<sub>4</sub> and R<sub>5</sub> each represents a member selected from the group consisting of a hydrogen atom and a sulfo group.

3. A photographic gelatino-silver-bromide emulsion sensitized with a supersensitizing combination of at least one dicarbocyanine dye selected from the class represented by the following general formula:



wherein R and R<sub>1</sub> each represents a lower alkyl group containing from 1 to 2 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and at least one compound containing at least one s-triazine ring.

oxazole series, those of the naphthoxazole series, those of the benzoselenazole series, those of the naphthoselenazole series, those of the 2-quinoline series, those of the 4-quinoline series, those of the benzimidazole series, and those of the 5,6-benzoquinoline series, and at least one triazine compound selected from the class represented by the following general formula:



wherein D and D<sub>1</sub> each represents a s-triazin-2-yl nucleus.

4. A photographic silver halide emulsion sensitized with a supersensitizing combination of at least one dicarbocyanine dye selected from the class represented by the following general formula:



wherein R and R<sub>1</sub> each represents an alkyl group containing from 1 to 4 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, those of the naphthoselenazole series, those of the 2-quinoline series, those of the 4-quinoline series, those of the benzimidazole series, and those of the 5,6-benzoquinoline series, and at least one triazine compound selected from the class represented by the following general formula:



wherein  $R_2$ ,  $R_3$ ,  $R_6$  and  $R_7$  each represents a member selected from the group consisting of a hydrogen atom, a hydroxyl group, an aryloxyl group, an alkoxy group, a halogen atom, a heterocyclic radical, an alkylthio group, an arylthio group, and an amino group, and  $R_4$  and  $R_5$  each represents a member selected from the group consisting of a hydrogen atom and a sulfo group.

5. A photographic gelatino-silver-bromide emulsion sensitized with a supersensitizing combination of at least one dicarboxcyanine dye selected from the class represented by the following general formula:



wherein R and R<sub>1</sub> each represents an alkyl group containing from 1 to 2 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the

group consisting of those of the benzothiazole series, those of the naphthothiazole series, those of the benzoxazole series, those of the naphthoxazole series, those of the benzoselenazole series, those of the naphthoselenazole series, those of the 2-quinoline series, those of the 4-quinoline series, those of the benzimidazole series, and those of the 5,6-benzoquinoline series, and at least one triazine compound selected from the class represented by the following general formula:

10



wherein  $D$  and  $D_1$  each represents a *s*-triazin-2-yl nucleus.

6. A photographic silver halide emulsion sensitized with a supersensitizing combination of at least one dicarboxylic dye selected from the class represented by the following general formula:



23 wherein R and  $R_1$  each represents an alkyl group containing from 1 to 4 carbon atoms,  $n$  represents a positive integer of from 1 to 2, X represents an acid radical,

30 Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzo-

35 selenazole series, and those of the naphthoselenazole series, and  $Z_1$  represents the non-metallic atoms necessary to complete a heterocyclic nucleus selected from the group consisting of those of the benzothiazole series, those

of the naphthothiazole series, those of the benzoxazole series, those of the naphthoxazole series, those of the benzoselenazole series, those of the naphthoselenazole series, those of the 2-quinoline series, those of the 4-

quinoline series, those of the benzimidazole series, and those of the 5,6-benzoquinoline series, and at least one triazine compound selected from the class represented by 45 the following general formula:



wherein  $R_2$ ,  $R_3$ , and  $R_6$  each represents a member selected from the group consisting of a hydrogen atom, a hydroxyl group, an aryloxyl group, an alkoxy group, a halogen atom, a heterocyclic radical, an alkylthio group, an arylthio group, and an amino group.

7. A photographic gelatino-silver-bromiodide emulsion sensitized with a supersensitizing combination of at least one dicarbocyanine dye selected from the class represented by the following general formula:



65 wherein R and  $R_1$  each represents an alkyl group containing from 1 to 2 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and  $Z_1$  represents the non-metallic atoms necessary to complete a heterocyclic nucleus selected from the group

consisting of those of the benzothiazole series, those of the naphthothiazole series, those of the benzoxazole series, those of the naphthoxazole series, those of the benzoselenazole series, those of the naphthoselenazole series, those of the 2-quinoline series, those of the 4-quinoline series, those of the benzimidazole series, and those of the 5,6-benzoquinoline series, and at least one triazine compound selected from the class represented by the following general formula:



wherein  $R_2$ ,  $R_3$ , and  $R_6$  each represents a member selected from the group consisting of a hydrogen atom, a hydroxyl group, an aryloxyl group, an alkoxy group, a halogen atom, a heterocyclic radical, an alkylthio group, an arylthio group and an amino group.

8. A photographic gelatino-silver-halide developing-out emulsion sensitized with a supersensitizing combination of a dicarbocyanine dye selected from the class represented by the following general formula:



wherein  $R$  and  $R_1$  each represents an alkyl group containing from 1 to 2 carbon atoms,  $X$  represents an acid radical,  $Z$  represents the non-metallic atoms necessary to complete a heterocyclic nucleus of the benzothiazole series and  $Z_1$  represents the non-metallic atoms necessary to complete a heterocyclic nucleus of the benzoxazole series, and at least one triazine compound selected from the class represented by the following general formula:



wherein  $D$  and  $D_1$  each represents a s-triazin-2-yl nucleus.

9. A photographic gelatino-silver-halide developing-out emulsion sensitized with a supersensitizing combination of 3,3'-diethyloxathiadicarbocyanine iodide and at least one bis(s-triazin-2-ylamino)biphenyl compound selected from the class represented by the following general formula:



wherein  $D$  and  $D_1$  each represents a s-triazin-2-yl nucleus.

10. A photographic gelatino-silver-halide developing-out emulsion sensitized with a supersensitizing combination of 3,3'-diethyloxathiadicarbocyanine iodide and 4,4'-bis[(2,4-di- $\beta$ -hydroxyethylamino)-s-triazin-2-ylamino]biphenyl-2,2'-disulfonic acid.

11. A photographic gelatino-silver-halide developing-out emulsion sensitized with a supersensitizing combination of a dicarbocyanine dye selected from the class represented by the following general formula:



wherein  $R$  and  $R_1$  each represents an alkyl group containing from 1 to 2 carbon atoms,  $X$  represents an acid radical,  $Z$  represents the non-metallic atoms necessary to complete a heterocyclic nucleus of the benzothiazole series and  $Z_1$  represents the non-metallic atoms necessary to complete a heterocyclic nucleus of the benzoxazole

series, and at least one triazine compound selected from the class represented by the following general formula:



wherein  $D$  and  $D_1$  each represents a s-triazin-2-yl nucleus.

12. A photographic gelatino-silver-halide developing-out emulsion sensitized with a supersensitizing combination of 3,3'-diethyloxathiadicarbocyanine iodide and 2,8-bis[4-(4-sulfoanilino)-6-hydroxy-s-triazin-2-ylamino]carbazole.

13. A photographic gelatino-silver-halide developing-out emulsion sensitized with a supersensitizing combination of a dicarbocyanine dye selected from the class represented by the following general formula:



wherein  $R$  and  $R_1$  each represents an alkyl group containing from 1 to 2 carbon atoms,  $X$  represents an acid

25 radical,  $Z$  represents the non-metallic atoms necessary to complete a heterocyclic nucleus of the benzothiazole series and  $Z_1$  represents the non-metallic atoms necessary to complete a heterocyclic nucleus of the benzoxazole series, and at least one triazine compound selected from

30 the class represented by the following general formula:



wherein  $R_2$ ,  $R_3$ , and  $R_6$  each represents a member selected from the group consisting of a hydrogen atom, a hydroxyl

40 group, an aryloxyl group, an alkoxy group, a halogen atom, a heterocyclic radical, an alkylthio group, an arylthio group, and an amino group.

14. A photographic gelatino-silver-halide developing-out emulsion sensitized with a supersensitizing combination of 3,3'-diethyloxathiadicarbocyanine iodide and 2-(2-benzothiazylamino)-4,6-dichloro-s-triazine.

15. A photographic gelatino-silver-halide developing-out emulsion sensitized with a supersensitizing combination of a dicarbocyanine dye selected from the class represented by the following general formula:



55 wherein  $R$  and  $R_1$  each represents an alkyl group containing from 1 to 2 carbon atoms,  $X$  represents an acid radical,  $Z$  represents the non-metallic atoms necessary to complete a heterocyclic nucleus of the benzothiazole series and  $Z_1$  represents the non-metallic atoms necessary to complete a heterocyclic nucleus of the benzoxazole series, and at least one triazine compound selected from

60 the class represented by the following general formula:



wherein  $D$  and  $D_1$  each represents a s-triazin-2-yl nucleus.

16. A photographic gelatino-silver-halide developing-out emulsion sensitized with a supersensitizing combination of 3,3'-diethyloxathiadicarbocyanine iodide and 4,4'-bis[(4,6-dihydroxy-s-triazin-2-ylamino)diphenyl]-2,2'-disulfonic acid.

17. A photographic gelatino-silver-halide developing-out emulsion sensitized with a supersensitizing combina-

75

tion of a dicarbocyanine dye selected from the class represented by the following general formula:



wherein R and R<sub>1</sub> each represents an alkyl group containing from 1 to 2 carbon atoms, X represents an acid radical, Z and Z<sub>1</sub> each represents the non-metallic atoms necessary to complete a heterocyclic nucleus of the benzoselenazole series, and at least one triazine compound selected from the class represented by the following general formula:



wherein R<sub>2</sub>, R<sub>3</sub>, and R<sub>6</sub> each represents a member selected from the group consisting of a hydrogen atom, a hydroxyl group, an aryloxyl group, an alkoxy group, a halogen atom, a heterocyclic radical, an alkylthio group, an arylthio group, and an amino group.

18. A photographic gelatino-silver-halide developing-out emulsion sensitized with a supersensitizing combination of 3,3'-diethylselenadicarbocyanine bromide and 1,4-bis[4-(4-anilino-6-β-hydroxyethylamino-s-triazin-2-ylamino)-2-sulfonyl]benzene.

19. A photographic silver halide emulsion capable of producing a dye image comprising a photographic silver halide emulsion containing (1) a dispersion of a phenol color-forming compound capable of coupling with the oxidation products of a primary aromatic amine developing agent to produce a cyan image, (2) a dicarbocyanine dye selected from the class represented by the following general formula:



wherein R and R<sub>1</sub> each represents an alkyl group containing from 1 to 4 carbon atoms, n represents a positive integer of from 1 to 2, X represents an acid radical, Z represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, and those of the naphthoselenazole series, and Z<sub>1</sub> represents the non-metallic atoms necessary to complete a heterocyclic nucleus selected from the group consisting of those of the benzothiazole series, those of the naphthothiazole series, those of the benzoxazole series, those of the naphthoxazole series, those of the benzoselenazole series, those of the naphthoselenazole series, those of the 2-quinoline series, those of the 4-quinoline series, those

of the benzimidazole series, and those of the 5,6-benzoquinoline series, and (3) a compound containing at least one s-triazine ring.

20. A photographic silver halide emulsion capable of producing a dye image, comprising a photographic silver halide emulsion containing (1) a dispersion of a color-forming compound selected from the class consisting of a phenol compound and a pyrazolone compound, capable of reacting with the oxidation products of a primary aromatic amine developing agent to form a cyan dye image and a magenta dye image, respectively, and (2) a s-triazine compound selected from the class consisting of those represented by the following two general formulas:



20 and



30 wherein R<sub>2</sub>, R<sub>3</sub>, R<sub>6</sub> and R<sub>7</sub> each represents a member selected from the group consisting of a hydrogen atom, a hydroxyl group, an aryloxyl group, an alkoxy group, a halogen atom, a heterocyclic radical, an alkylthio group, an arylthio group, and an amino group, and R<sub>4</sub> and R<sub>5</sub> each represents a member selected from the group consisting of a hydrogen atom and a sulfo group, said s-triazine compound being incapable of reacting with the oxidation products of a primary aromatic amine developing agent to form a dye image.

40

#### References Cited in the file of this patent

#### UNITED STATES PATENTS

- |           |                |       |                |
|-----------|----------------|-------|----------------|
| 2,271,623 | Carroll        | ----- | Feb. 3, 1942   |
| 2,397,867 | Jennings       | ----- | Apr. 2, 1946   |
| 2,418,747 | Bavley         | ----- | Apr. 8, 1947   |
| 2,422,080 | Collins et al. | ----- | June 10, 1947  |
| 2,476,536 | Dersch         | ----- | July 19, 1949  |
| 2,701,198 | Carroll        | ----- | Feb. 1, 1955   |
| 2,718,466 | Wolfson        | ----- | Sept. 20, 1955 |

#### FOREIGN PATENTS

- |         |               |       |               |
|---------|---------------|-------|---------------|
| 675,656 | Great Britain | ----- | July 16, 1952 |
| 832,391 | Germany       | ----- | Feb. 25, 1952 |

#### OTHER REFERENCES

- Mees: "The Theory of the Photographic Process," MacMillan Co., N.Y., 1954, page 365.